

## UNITED STATES PATENT OFFICE

2,401,900

## SOUND RECORDING COMPOSITION

Horace P. Billings, Haddonfield, N. J., assignor to  
 Radio Corporation of America, a corporation of  
 Delaware

No Drawing. Application October 29, 1943,  
 Serial No. 508,250

2 Claims. (Cl. 106—37)

1

This invention relates to a composition of matter and to the method of preparing the same, and more particularly to a composition of matter suitable for use as a sound recording material.

Compositions of montan wax and stearic acid in the form of metallic soaps of sodium and lead have constituted recording wax-like compositions for many years. The gel-forming nature of these soaps is well known; and when the soap ratio of uncombined fatty acid is balanced, films of approximately 0.020" to 0.030" thick assume a lustrous surface suitable for use in sound recording. Heretofore, the flowing quality of such compositions has been controlled by temperature adjustments, and this has been relied upon to obtain level surfaces of the composition. In some cases, it is desirable to flow the wax-like composition onto a suitable base, such as glass, metal or the like in the form of a very thin film which forms the recording surface. In such cases, obviously, the film must be of uniform thickness and entirely level. The flow characteristics of the prior art compositions are not such as to afford even flow for very thin films.

The primary object of my present invention is to provide an improved composition of matter suitable for use in sound recording and free from the aforementioned difficulty.

More particularly, it is an object of my present invention to provide an improved composition of matter as aforesaid which will flow out uniformly and evenly even in very thin film layers.

A further object of my present invention is to provide a method of preparing the improved composition of my present invention.

Another object of my present invention is to provide an improved composition of matter and method as aforesaid which will be highly efficient in use and which can be practiced even by those not highly skilled in the art of flowing wax.

In accordance with my present invention, I incorporate into a suitable metallic soap base a plasticizer comprising a mixture of a wax, a mineral oil, and free stearic acid. The wax may be either of vegetable or animal origin, as more fully set forth hereinafter. Preferably, the soap stock is first made up, after which the wax and mineral oil are preferably first added thereto, the free stearic acid being added as the last ingredient.

In practicing the present invention, the soap stock or base may be made up of sodium and lead compounded with a mixture of stearic acid, and montan wax. The montan wax to stearic acid ratio may vary between the proportions of 1 to 2.3 and 1 to 3. The sodium and lead, in chemical

2

combination, may vary between the proportions of 1 to 1.5 and 1 to 3.5. In a typical formula, the soap stock mixture may be compounded of 30 per cent montan wax (having an acid value of 80 to 82 milligrams of potassium hydroxide per gram of wax), 60 per cent stearic acid, 2.5 per cent to 3 per cent sodium and 5.5 to 8.5 per cent lead. These percentages are based on the finished stock which constitutes a metallic soap base, and the stock may be prepared according to well known methods practiced in the art.

To impart to the soap stock the desired flow characteristics, I then incorporate into it a plasticizer consisting of a mixture of a suitable wax, a mineral oil, and free stearic acid. The wax may comprise an animal wax, such as spermaceti, or a wax such as that sold under the trade name "Ceranova" wax, which is manufactured by the Avon Importing Company, New York city, and consists of a vegetable wax of amorphous nature. I have found that a plasticizer made up in the following proportions gives excellent results:

Ceranova wax—approximately 18 per cent.  
 White mineral oil—approximately 57 per cent.  
 Stearic acid (triple pressed)—approximately 25 per cent.

The above materials forming the plasticizer are added preferably in a particular sequence. First, the Ceranova wax and the white mineral oil are melted together and are clarified. This liquid mixture is then added with stirring to the liquid soap stock which is maintained at a temperature in the neighborhood of 140° C. After this mixture has been well stirred, and while still maintaining the stock at about 140° C., the stearic acid is added in melted form and the entire mixture is well stirred to produce a homogeneous mixture. The finished composition may then be cast into forms in suitable molds, and subsequently remelted for flowing in thin, uniform films on glass, metal, or other suitable surfaces.

The amount of improved plasticizer according to my present invention which is added to the base or soap stock constitutes between 8 per cent to 10 per cent by weight of the finished composition. The sound recording material produced as above described is much more glossy than similar prior art compositions and has far less tendency to fog after cooling in the form of a film. Also, a record made of the composition according to my present invention will be found to be extremely accurate and will result in more faithful reproduction of the original sounds.

Although I have shown and described but one

form of my invention and one method of preparing the same, it will undoubtedly be obvious to those skilled in the art that many changes in both are possible within the spirit of the present invention. I therefore desire that my invention shall not be limited except insofar as is made necessary by the prior art and by the spirit of the appended claims.

I claim as my invention:

1. A composition of matter suitable for use in recording sound which comprises a base of a metallic soap in which is incorporated a plasticizer comprising a mixture of a wax, a mineral oil and free stearic acid, said mixture containing

approximately 18 percent wax, approximately 57 percent mineral oil and approximately 25 percent stearic acid by weight.

2. The method of preparing a composition of matter suitable for use as a sound recording material which comprises preparing a base stock of one or more metallic soaps, and thereafter adding to said stock a plasticizer adapted to enhance the flow characteristics of said stock in relatively thin films, said plasticizer comprising a mixture of a wax, a mineral oil and stearic acid, and said wax and mineral oil being added to said stock prior to adding the stearic acid thereto.

HORACE P. BILLINGS.